

Feb. 10, 1931.

M. M. AUSTIN

1,791,785

TANTALUM SPINNERET

Original Filed June 2, 1928

Fig. 1.



Fig. 2.



Inventor  
Miner M. Austin.

By Williams, Bradbury, McColl  
F. Hiddle. Atty's.

## UNITED STATES PATENT OFFICE

MINER M. AUSTIN, OF WAUKEGAN, ILLINOIS, ASSIGNOR TO FANSTEEL PRODUCTS COMPANY, INC., OF NORTH CHICAGO, ILLINOIS, A CORPORATION OF ILLINOIS

## TANTALUM SPINNERET

Application filed June 2, 1928, Serial No. 282,400. Renewed October 27, 1930.

This invention relates to spinnerets and pertains more particularly to an improved spinneret of tantalum which is coated by a hard electrolytic film whereby the minute 5 openings are not distorted or worn out of shape by continued usage. The object of this invention is to provide a spinneret which will not be corroded either in the fluids in which the spinneret is finally used or in the 10 fluid used to dissolve the cores in obtaining the minute openings.

A further object is to provide a spinneret with a hard enamel-like film whereby the shape of the openings are not irregularly 15 worn.

Other objects of my invention will be apparent as the detailed description of my invention proceeds.

A preferred embodiment of the invention 20 is illustrated in the accompanying drawing wherein similar parts are designated by like reference characters throughout the several views and wherein

Fig. 1 is a perspective of my improved 25 spinneret having a portion broken or cut away to show the construction thereof.

Fig. 2 is a diagrammatic representation of the film forming bath.

The manufacture of artificial silk or rayon 30 requires the use of spinnerets which have very fine openings and in which the openings are circular. If the openings are distorted or flat the rayon produced will be of an inferior quality and will only demand about 35 one-third of the market price.

Heretofore such spinnerets have been made of platinum, platinum gold alloys, etc., because these were the only metals known which combined suitable acid resisting qualities 40 with a malleability and hardness which would permit the drilling of the extremely small holes and which would prevent these holes from being deformed by usage. Tantalum had been tried without success because the 45 metal was so hard that the holes could not be properly drilled. If the metal were softened or annealed to overcome this difficulty the holes were likely to be deformed by subsequent use.

50 I have discovered that by coating the spin-

neret with an electrolytic film, a hard enamel-like surface is formed thereon which is of infinitesimal thickness, but which, nevertheless, is extremely resistant and which renders the spinneret practically impervious to corrosive action and to the erosion or wearing away due to continued usage. 55

In Fig. 1 I have shown a spinneret 10 of conventional type which is provided with a face plate 11 in which are drilled a plurality 60 of holes 13.

Since the tantalum must be relatively malleable to permit forming the holes 13 therein, it is necessary that its surface be hardened if it is to resist the wear to which it must be subjected. To accomplish this I immerse the spinneret in sulphuric acid bath (specific gravity about 1.250), and subject it to an electric potential of about 20 to 110 volts. The time of immersion will necessarily vary with 70 the immersed area of the spinneret but I have found that by using alternating current of 110 volts the proper film is formed on an area of 10 square inches by subjecting it to this potential for about 30 seconds, a resistance 75 of about 80 ohms being in the circuit as shown in Fig. 6.

A simple apparatus for electrolytically filming the spinneret consists of a suitable metallic receptacle 18 containing sulphuric acid 19. The container is connected by a conductor 20 to an alternating current source 21 which is, in turn, connected by conductor 22 to variable resistance 23, this resistance being connected by conductor 24 to the spinneret as shown in Fig. 6. The resistance in my preferred embodiment is about 80 ohms and the alternating current source is 110 80 volts. 85

It is understood, however, that a direct 90 current may be used instead of an alternating current and that various changes in the method of forming may be made without departing from the spirit of my invention.

A somewhat thicker film and one that may be somewhat more durable may be formed on the finished spinneret by heating it gently, say to 300° C. in air, preferably in an electric furnace. 95

The tantalum 11 is covered by a film 17 of 100

infinitesimal thickness, said film also serving to protect the openings in the face of the spinneret as shown in Fig. 1. The electrolytic film not only increases the hardness and wear resistance of the metal but it provides a highly decorative film of vari-colored iridescent nature, which is characteristic of this metal. The decorative feature, however, forms no part of the present invention.

10 While I have described a preferred embodiment of my invention it is understood that I am not limited to the details thereof, except as confined by the following claim.

I claim:

15 An article of manufacture comprising a tantalum spinneret and a hard resistant oxide film formed directly thereon whereby said tantalum spinneret is protected against corrosion and wear.

20 In witness whereof, I hereunto subscribe my name this 24th day of May, 1928.

MINER M. AUSTIN.

85

30

85

40

45

50

55

60

65